# EUROPEAN PATENT SPECIFICATION

(11) **EP 1 742 753 B1**
(45) Date of publication and mention of the grant of the patent: **30.07.2008**
(21) Application number: 99935265.1
(22) Date of filing: 19.07.1999
(51) Int. Cl.: B22F 1/00, C22C 33/02

(54) **ALLOYED, NON-OXIDISING METAL POWDER**
LEGIERTES, NICHTOXIDIERENDES METALLPULVER
POUDRE METALLIQUE ALLIEE NON OXYDANTE

(30) Priority: 06.08.1998 SE 9802682
(43) Date of publication of application: 17.01.2007
(62) Divisional of application: 08153706.0
(73) Proprietor: Rutger Larsson Konsult AB, 264 91 Klippan (SE)
(72) Inventor: LARSSON, Rutger, S-264 91 Klippan (SE); AXMIN, Erik, S-264 35 Klippan (SE)
(74) Representative: Karlsson, Leif Karl Gunnar
(86) International application number: PCT/SE1999/001293
(87) International publication number: WO 2000/007759

(56) References cited:
- WO-A1-96/05007
- WO-A1-97/41986
- DE-B- 2 220 673
- JP-A- 61 276 949
- US-A- 5 522 914
- US-A1- 9 302 818

## Description

The present invention relates to an atomised, non-oxidising, alloyed metal powder based on iron enriched with carbide-bound carbon in the surface layer, and also to the use of the atomised, non-oxidising, alloyed metal powder.

Most metal powders are produced by means of atomising, electrolysis or through chemical or oxide reduction. Powder is used in mixtures for producing alloy compositions that are bound metallurgically upon sintering. Metallic and non-metallic powders can be combined to produce composite material having special properties.

The powder metallurgical composition most frequently used is iron powder, which is used in the manufacture of various structured parts. Iron powder is sometimes used alone or, which is more usual, together with various additives in order to improve the mechanical properties of compacted sintered products. Powder additives include carbon, copper, nickel and molybdenum.

US, A, 5,522,914 reveals an alloyed metal powder composed of 0.80 to 3.00 per cent by weight carbon, 0.20 to 2.00 per cent by weight manganese, 0.20 to 1.50 per cent by weight silicon, as well as 3.0 to 12.0 per cent by weight chromium, 0.20 to 0.30 per cent by weight sulphur, up to 0.04 per cent by weight phosphorous, 0.25 to 10.0 per cent by weight vanadium, up to 11.0 per cent by weight molybdenum, up to 18.00 per cent by weight mercury, up to 10 per cent by weight cobalt and up to 0.10 per cent by weight nitrogen, besides the iron. The oxygen content in the powder is less than 0.025 per cent by weight. The powder is produced by atomisation in nitrogen gas atmosphere in order to achieve a low oxygen content.

The problem in the production of metal powder is the oxygen content. A high oxygen content is unsuitable when metal powder is to be used for tools or other articles requiring high mechanical strength. In US, A, 5,522,914 the problem has been solved by atomising the powder in nitrogen gas atmosphere. This is expensive and results in undesired nitrogen being included in the alloyed powder produced.

The problem of the added nitrogen is solved by using hydrocarbon which is partially carbonised during the atomisation process. Such use of hydrocarbon is known through Swedish patent application 9601482-4. The atomised steel powder obtained has acquired enriched carbide-bound carbon in the surface layer, and a low oxygen content.

It has now surprisingly been found that oxidation can be prevented by enriching the carbide-bound carbon in the surface layer. This means that alloyed powder particles can be produced that include oxidation-sensitive alloying substances such as chromium, manganese, silicon. Furthermore, the use of nitrogen gas atmosphere can be avoided since the atmosphere in the atomising equipment is saturated with vaporised or carbonised atomising medium.

The present invention thus solves the problems of added oxygen and undesired nitrogen. The atomised, alloyed metal powder according to the invention is non-oxidising as well as preventing oxidation. It has improved powder-metallurgical properties such as strength and toughness. The carbide-bound carbon in the surface layer of the powder particles is enriched.

### Detailed description of the invention

The non-oxidising, alloyed metal powder in accordance with the invention is given in claim 1. It comprises oxidation-sensitive alloying metals such as chromium and manganese, besides iron and carbide-bound carbon. These alloying metals are also capable of carbide-binding carbon.

Atomising medium used in the producion of the non-oxidising alloyed metal powder consists of hydrocarbons selected from the group comprising paraffin, diesel oils, or other cyclic or acyclic hydrocarbons that have been partially carbonised during the atomisation. Hydrogen gas is formed during the carbonisation of the hydrocarbons, as well as the carbides that are bound to the metals in the powder particles. The atmosphere in the atomising vessel is saturated with vaporised or carbonised atomising medium consisting of hydrocarbons and hydrogen gas. The atmosphere is thus reducing, thereby protecting the powder particles produced.

The invention provides atomised, alloyed, non-oxidising metal powder based on iron with enriched carbide-bound carbon in the surface layer, that has been carbide-bound to the metal in the powder particles by carbonised atomising medium selected from the group comprising paraffin, diesel oils, or other cyclic or acyclic hydrocarbons during the atomising.

The size distribution in the powder particles is 45 to 200 µm.

Producing the atomised, alloyed, non-oxidising metal powder, based on iron with enriched carbide-bound carbon in the surface layer enables the manufacture of compacted sintered products such as toothed wheels, ball-bearings and tool steel. These products require high mechanical strength and toughness, and these properties are achieved since the alloying additives increase tempering quality and strength. The products are manufactured by means of conventional powder metallurgical compressing, hot compacting and sintering, hot isostatic pressing and sinter forging.

Since the metal powder produced is non-oxidising and prevents oxidation it can be mixed with other powder produced from oxidation-sensitive metals. This enables the manufacture of composite material having completely new qualities.

The present invention thus also relates to the use of the atomised, alloyed, non-oxidising metal powder as claimed in claim 1 for the manufacture of compressed, sintered products, such as toothed wheels, ball-bearings, tool steel, manufactured by means of conventional powder-metallurgical compression, hot compacting and sintering, hot isostatic compacting and sinter forging.

The present invention will be further illustrated with concrete examples which should not, however, be considered as limiting the scope of protection of the invention otherwise than as defined in the appended claims.

In the following example, alloyed, non-oxidising metal powder according to the invention was produced in accordance with the procedure described in Swedish patent application No. 9601482-4. Paraffin was used as atomising medium in the experiments.

### Example

An alloyed metal powder with metal carbides in the surface layer was produced having 8.0 to 10 per cent by weight chromium, 8.0 to 10 per cent by weight manganese, 0.8 to 1.2 per cent by weight carbon and the remainder iron. The powder produced is spherical and has a size distribution of between 45 and 200 µm.

## Claims

1. An atomised, alloyed, non-oxidising metal powder based on iron enriched with carbide-bound carbon in the surface layer, that has been carbide-bound to the metals by carbonised atomised medium selected from the group comprising paraffin, diesel oils, or other cyclic or acyclic hydrocarbons **characterised in that** besides iron and the carbide bound carbon, the powder particles comprise 8.0-10% by weight of chromium, 8.0-10% by weight of manganese, 0.8-1.2% by weight of carbon and the remainder iron and **in that** the oxygen content is less than 200 ppm, and **in that** the particles are spherical and has a size distribution of between 45 and 200 µm.

2. Use of the atomised, alloyed, non-oxidising metal powder according to claim 1 for the manufacture of compressed, sintered products such as toothed wheels, ball-bearings, tool steel, manufactured by means of conventional powder-metallurgical compression, hot compacting and sintering, hot isostatic compacting and sinter forgoing.

3. Use of the atomised, alloyed, non-oxidising metal powder according to claim 1 for the manufacture of compressed, sintered alloyed products such a toothed wheels, ball-bearings, tool steel, together with iron powder.

## Patentansprüche

1. Zerstäubtes, legiertes, nicht-oxidierendes Metallpulver, basierend auf Eisen, angereichert mit als Carbid gebundenem Kohlenstoff in der Oberflächenschicht, welches durch carbonisiertes, zerstäubtes Medium, ausgewählt aus der Gruppe, bestehend aus Paraffin, Dieselölen oder anderen zyklischen oder azyklischen Kohlenwasserstoffen, als Carbid an die Metalle gebunden wurde, **dadurch gekennzeichnet, daß** die Pulverpartikel neben Eisen und dem als Carbid gebundenen Kohlenstoff 8,0-10 Gewichts-% Chrom, 8,0-10 Gewichts-% Mangan, 0,8-1,2 Gewichts-% Kohlenstoff und Rest Eisen umfassen und daß der Sauerstoffgehalt weniger als 200 ppm beträgt und daß die Partikel kugelförmig sind und eine Größenverteilung zwischen 45 und 200 µm aufweisen.

2. Verwendung des zerstäubten, legierten, nicht-oxidierenden Metallpulvers nach Anspruch 1 für die Herstellung von komprimierten gesinterten Produkten, wie Zahnrädem, Kugellagem, Werkzeugstahl, hergestellt unter Verwendung von konventioneller pulvermetallurgischer Kompression, Heißkompaktierung und Sintem, heißisostatischem Pressen und Sinterschmieden.

3. Verwendung des zerstäubten, legierten, nicht-oxidierten Metallpulvers nach Anspruch 1 für die Herstellung von komprimierten gesinterten Legierungsprodukten, wie Zahnrädern, Kugellagern, Werkzeugstahl, zusammen mit Eisenpulver.

## Revendications

1. Une poudre métallique alliée, atomisée, non oxydante, à base de fer enrichi en carbone lié au carbure dans la couche de surface, qui a été liée au carbure avec les métaux par un milieu atomisé, carbonisé, sélectionné dans le groupe comprenant de la paraffine, des huiles diesel, ou d'autres hydrocarbures cycliques ou acycliques, **caractérisée en ce que** hormis le fer et le carbone lié au carbure, les particules de poudre comportent 8.0 - 10 % en poids de chrome, 8.0 - 10 % en poids de manganèse, 0.8 - 1.2 % en poids de carbone et le reste en fer et **en ce que** la teneur en oxygène est inférieure à 200 ppm, et **en ce que** les particules sont sphériques et ont une répartition granulométrique variant entre 45 et 200 µm.

2. L'utilisation de la poudre métallique alliée, atomisée, non oxydante, selon la revendication 1 pour la fabrication de produites frittés, compressés, notamment des roues dentées, paliers à billes, acier à outils, fabriqués au moyen de compression conventionnelle par métallurgie des poudres, compaction à chaud et frittage, compaction isostatique à chaud et pressage à chaud.

3. L'utilisation de la poudre métallique alliée, atomisée, non oxydante, selon la revendication 1 pour la fabrication de produits alliés frittés, compressés, notamment des roues dentées, paliers à billes, acier à outils, conjointement avec de la poudre de fer.
